

Sept. 1, 1959

W. H. ROSS, JR

2,901,821

ALUMINUM COATED WITH ALUMINUM BENZOATE, AND METHOD  
AND COMPOSITION FOR MAKING SAME  
Filed Nov. 18, 1955



INVENTOR.  
*Willford H. Ross Jr.*

BY

*Paul & Paul*

ATTORNEYS.

# United States Patent Office

2,901,821

Patented Sept. 1, 1959

1

2,901,821

## ALUMINUM COATED WITH ALUMINUM BENZOATE, AND METHOD AND COMPOSITION FOR MAKING SAME

Wilford H. Ross, Jr., Detroit, Mich., assignor to Detrex Chemical Industries, Inc., Detroit, Mich., a corporation of Michigan

Application November 18, 1955, Serial No. 562,368

11 Claims. (Cl. 29—495)

This invention relates to the application of protective coatings to aluminum or aluminum alloys, and more particularly relates to compositions and methods for inhibiting an aluminum surface against atmospheric oxidation. More particularly, this invention relates to the removal of oxide from an aluminum surface combined with the formation on such surface of a tightly adherent coating which resists atmospheric oxidation and which does not interfere with the welding of the metal.

It is an object of this invention to provide a coating which has the advantageous characteristics just referred to. Still another object is to provide a method of applying such a coating to aluminum or its alloys. Still another object is to provide a method of removing an oxide film from an aluminum surface and for also applying to such surface a chemical coating which protects the aluminum against atmospheric oxidation.

In the fabrication of aluminum articles, it is conventional to assemble prefabricated aluminum pieces by welding. However, aluminum has a much higher electrical conductivity than most of the other weldable metals. This necessitates the use of welders of high capacity which are capable of supplying the high current necessary for welding aluminum.

Aluminum combines almost instantaneously with atmospheric oxygen to form a crystalline aluminum oxide on the aluminum surface which has both a high and erratic electrical resistance. This in turn affects the amount of heat produced at the weld resulting in wide variation in weld strengths unless this oxide is removed prior to welding. This disadvantage is particularly felt when the aluminum is to be spot-welded.

It is accordingly necessary to clean and deoxidize the aluminum surface to produce welds of consistent high strength, good appearance, minimum indentation, and maximum reliability. Conventional production practice is to clean the aluminum article in a suitable cleaning medium, usually an inhibited alkaline cleaner, and then mechanically or chemically to deoxidize the surface. This results in a surface having a contact resistivity of 20 to 100 microhms.

Conventional chemical deoxidizers are selected from the class of strong acids; they usually consist of sulfuric acid, chromic acid, nitric acid or phosphoric acid or a combination of these acids, or their sodium salts suitably acidified to a low pH range or high acid content. These strongly acid chemicals, however, not only remove the oxide layer but also attack the underlying aluminum. In attacking the aluminum, a second film is produced on the surface which sometimes has as high an electrical resistance as the original oxide layer. Therefore, time of exposure to such treatment is critical.

A number of proprietary products are offered the trade which contain inhibitors to this subsequent attack on the basic aluminum surface. Included among such inhibitors are hydrofluosilicic, hydrofluoric or fluoroboric acids or other fluorine-containing materials which presumably react with any freed aluminum to form insoluble aluminum silicofluoride, fluoride, etc., which act as a passivating layer to further attack. These compounds have the

2

disadvantage, however, of increasing contact resistance and affecting the alloying character of the "nugget" or weld since they are not volatilized at the weld. A further disadvantage of the strong acid deoxidizers is that special, expensive articles of equipment, including corrosion-resistant tanks, are necessary. Moreover, personnel hazards are involved in the use of strongly acid chemicals.

It is accordingly another object of this invention to provide a method as discussed above using a solution which operates at a relatively high pH range, avoiding personnel hazards and also costly equipment.

Another object is to provide a method and solution which remove the crystalline oxide from an aluminum surface without seriously attacking or etching the underlying aluminum surface.

Still another object is to inhibit the treating solution so that if any free aluminum goes into solution, it immediately reacts to form a passivating layer on the surface of the aluminum.

Yet another object of this invention is to provide a coating for aluminum or its alloys which decomposes at a welding temperature with the production of gaseous products and does not affect the alloying nature of the weld.

Other objects and advantages of this invention will appear in further detail hereinafter, and in the drawing.

The drawing represents a perspective view of an aluminum article in accordance with this invention, having an aluminum benzoate coating thereon. The drawing is essentially a schematic representation of the surface coating, which is extremely thin and does not therefore lend itself to accurate illustration. The surface markings in the drawing are intended to illustrate a general roughness of the surface area, and are not intended to suggest that the aluminum benzoate coating consists of specks or the like, or that such coating is essentially discontinuous in nature. The aluminum benzoate coating is fine grained and covers the entire aluminum surface.

It has been found that the foregoing objects are obtained by reacting the aluminum surface with benzenoid carboxylic acid. This is preferably but not necessarily attained by providing a mixture of acid phosphates buffered to a pH range of 4.4 to 5.5 containing a small percentage of benzenoid carboxylic acid. One example of a suitable and preferred composition of matter is:

|                                                             | Percent by weight |
|-------------------------------------------------------------|-------------------|
| Monosodium phosphate                                        | 91.8              |
| Disodium phosphate                                          | 3.7               |
| Benzoic acid                                                | 2.5               |
| 50 Wetting agent (iso octyl, phenoxyethoxyethylene ethanol) | 2.0               |

The following approximate ranges of proportions are applicable in the practice of this invention:

|                                     | Percent by weight |
|-------------------------------------|-------------------|
| Alkali metal dihydrogen phosphate   | 85.0 to 95.0      |
| Alkali metal monohydrogen phosphate | 2.5 to 5.0        |
| Benzoic acid                        | 0.25 to 10.0      |

However, under some conditions, benzoic acid may be used independently of the acid phosphate chemicals.

The wetting agent, which may be varied considerably in form or chemical composition, or even entirely eliminated, assists in wetting the surface of the metal or oxide and facilitating chemical reactivity.

It is important to provide a solution which is buffered in the pH range 4.4-5.5. This can be accomplished by mixtures of dihydrogen and monohydrogen phosphates of sodium and the other alkali metals, including potassium or other alkali or ammonium salts, suitably buffered to a pH range of 4.4 to 5.5.

It has been further discovered that the inclusion of soluble alkali metal or ammonium chromates, dichro-

mates or chromic acid in this composition further improves its deoxidizing power without deterring from the activity of the oxidation inhibitor. This is caused by a coaction of phosphoric and chromic acids to deoxidize or dissolve aluminum oxide. The aluminum oxide is removed in an acidic medium buffered to a pH of 4.4 to 5.5, incorporating an inhibitor in the form of benzoic acid. A preferred composition of matter corresponding to this formula is as follows, this composition being specified by way of example only:

|                      | Percent by weight |
|----------------------|-------------------|
| Monosodium phosphate | 82.6              |
| Disodium phosphate   | 2.2               |
| Sodium dichromate    | 13.7              |
| Benzoic acid         | 1.5 15            |

The following approximate ranges of proportions are applicable in the practice of this invention when chromate is used:

|                                     | Percent by weight |
|-------------------------------------|-------------------|
| Alkali metal dihydrogen phosphate   | 75.0 to 90.0      |
| Alkali metal monohydrogen phosphate | 1.5 to 4.0        |
| Chromate (or chromic acid) as above | 5.0 to 15.0       |
| Benzoic acid                        | 0.25 to 10.0      |

Similarly, surface active agents may be added to the foregoing composition to facilitate wetting. This composition may likewise be duplicated by suitable neutralization of phosphoric acid with alkali metal hydroxide or mixtures of potassium or other alkali salts.

In use, these compositions are dissolved in water at a concentration of preferably from 8 to 16 ounces total chemicals per gallon of water, the latter figure usually being more desirable. Solution is preferably accomplished by heating to temperatures over 140°-160° F. Operating temperatures of the bath are in the range of 180°-200° F.

The aluminum part to be deoxidized and coated is usually pre-cleaned in an inhibited alkali solution followed by a water rinse, or by degreasing with trichloroethylene followed by an alkali cleaning treatment. The part is then immersed in the solution of the deoxidizer as heretofore defined, for about 5 to 10 minutes, and then water rinsed. Aluminum or aluminum alloy processed in this way has none of the objectionable etched appearance common with stronger acid deoxidizers but remains bright. The period of immersion in the bath should be limited, however, since immersion for an excessive period tends to produce a light brown or black discoloration, depending upon the alloy. This discoloration also indicates an excessive surface contact resistance. The appropriate immersion time can readily be obtained by visual observation.

Parts processed in the manner described herein have been found to resist atmospheric oxidation for longer periods of time than untreated aluminum.

Although this invention has been described with particular reference to the application of a coating to aluminum, it will be appreciated that the term "aluminum," as referred to herein, is intended to cover either wrought, cast, extruded, or any other form of aluminum, and is also intended to cover the various alloys of aluminum.

While this invention has particular advantages in connection with the preparation of aluminum for electric spot-welding, it will be appreciated that the coating as applied in accordance with this invention has a wide variety of other uses.

Various modifications may be made in the coating solution and in the method of applying the coating to the metal, including substitution of equivalents for the specific chemicals and method steps described in the foregoing specification, and further including the use of certain features of the invention independently of other features. All such modifications may be made without departing from the spirit or scope of this invention, as defined in the appended claims.

Having thus described my invention, I claim:

1. Method of welding aluminum or alloys thereof comprising chemically coating the aluminum surface with a thin film of aluminum benzoate, and then heating the aluminum and aluminum benzoate coating to welding temperature.

2. Method of coating aluminum or its alloys comprising immersing the aluminum in a dilute water solution containing dihydrogen phosphate coating chemicals and benzoic acid, said benzoic acid being present in a solution having a pH of about 4.4 to 5.5 and in a substantial quantity to react with said aluminum to form an aluminum benzoate coating.

3. Method of welding aluminum or an alloy thereof having aluminum oxide on the surface thereof comprising chemically coating the surface of said aluminum with aluminum benzoate, and heating the aluminum to welding temperature thereby decomposing the benzoate to form gaseous products while the aluminum is welded.

4. Method of welding aluminum or an aluminum alloy having aluminum oxide on the surface thereof comprising etching the aluminum with a benzoic acid solution having a pH of about 4.4 to 5.5, thereby dissolving the aluminum oxide and forming an integral coating of aluminum benzoate on the surface of said aluminum, and heating the aluminum to welding temperature thereby decomposing the aluminum benzoate as the aluminum is welded.

5. An article having an aluminum surface covered by a coating formed in situ on said surface by contacting and reacting said aluminum surface with a dilute aqueous solution of benzoic acid containing a buffer adjusting the solution pH to about 4.4 to 5.5, and comprising a substantially insoluble benzoate of aluminum.

6. An article having a surface of aluminum coated with a fine grained, strongly adherent coating formed integrally in situ on said surface by contacting and reacting said aluminum surface with a dilute aqueous solution of benzoic acid containing a buffer adjusting the solution pH to about 4.4 to 5.5, at least the major portion of said coating being benzoate and being substantially free of aluminum oxide.

7. A composition of matter for coating aluminum or its alloys to protect the metal against atmospheric oxidation prior to welding consisting essentially of an acidic aqueous solution of benzoic acid and alkali metal dihydrogen phosphate, said solution having a pH of about 4.4 to 5.5, and said benzoate being present in a substantial quantity to react with aluminum to form an aluminum benzoate coating.

8. A composition of matter for coating aluminum or its alloys to protect the metal against atmospheric oxidation prior to welding consisting essentially of an acidic aqueous solution of benzoic acid, alkali metal dihydrogen phosphate, and chromium compound selected from the group consisting of the chromates and dichromates and chromic acid, said solution having a pH of about 4.4 to 5.5, and said benzoic acid comprising about 0.25 to 10.0% by weight of the combined weight of benzoic acid and said phosphate.

9. Composition of matter for coating aluminum consisting essentially of:

|                                     | Percent by weight |
|-------------------------------------|-------------------|
| Benzoic acid                        | 0.25 to 10.0      |
| Alkali metal dihydrogen phosphate   | 85.0 to 95.0      |
| Alkali metal monohydrogen phosphate | 2.5 to 5.0        |

10. Composition of matter for coating aluminum consisting essentially of:

|                                                                                                                 | Percent by weight |
|-----------------------------------------------------------------------------------------------------------------|-------------------|
| Benzoic acid                                                                                                    | 0.25 to 10.0      |
| Alkali metal dihydrogen phosphate                                                                               | 75.0 to 90.0      |
| Alkali metal monohydrogen phosphate                                                                             | 1.5 to 4.0        |
| Chromate compound selected from the group consisting of alkali metal chromates and dichromates and chromic acid | 5.0 to 15.0       |

11. Method of applying a coating to aluminum or an alloy thereof comprising contacting and reacting the aluminum with a dilute aqueous solution of benzoic acid containing a buffer adjusting the solution pH to about 4.4 to 5.5.

2,052,278  
2,465,750  
2,494,910  
2,672,681

Callis et al. \_\_\_\_\_ Aug. 25, 1936  
Reid \_\_\_\_\_ Mar. 29, 1949  
Spruance \_\_\_\_\_ Jan. 17, 1950  
Kalin \_\_\_\_\_ Mar. 23, 1954

## FOREIGN PATENTS

Germany \_\_\_\_\_ Nov. 22, 1951  
Great Britain \_\_\_\_\_ Dec. 15, 1954

References Cited in the file of this patent

821,907  
720,276

UNITED STATES PATENTS

1,911,537 Tanner \_\_\_\_\_ May 30, 1933